

Feb. 24, 1959

R. S. DEAN

2,875,038

METHOD OF PRODUCING CRYSTALLINE METAL

Filed Feb. 16, 1955

3 Sheets-Sheet 1



Feb. 24, 1959

R. S. DEAN

2,875,038

METHOD OF PRODUCING CRYSTALLINE METAL

Filed Feb. 16, 1955

3 Sheets-Sheet 2



Feb. 24, 1959

R. S. DEAN

2,875,038

METHOD OF PRODUCING CRYSTALLINE METAL

Filed Feb. 16, 1955

3 Sheets-Sheet 3



# United States Patent Office

2,875,038

Patented Feb. 24, 1959

1

2,875,038

## METHOD OF PRODUCING CRYSTALLINE METAL

Reginald S. Dean, University Park, Md., assignor to Chicago Development Corporation, Riverdale, Md., a corporation of Delaware

Application February 16, 1955, Serial No. 488,540

2 Claims. (Cl. 75—84.5)

This invention relates to processes for producing titanium and zirconium. It is particularly concerned with processes for forming and reducing the lower chlorides of titanium and zirconium to produce pure, massive or coarsely particulate, titanium or zirconium in a form which is not pyrophoric or attacked by water or dilute acid. It has particular but not exclusive application to processes which are in whole or in part electrolytic.

The problem of producing titanium or zirconium in a massive or coarsely particulate form by the reduction of a solution of its lower chlorides in fused baths of alkaline chlorides or bromides has had considerable attention from investigators in the metallurgical field. The problem has been partially solved by several inventors but only by special means which are intrinsically unsatisfactory and uneconomical. The most successful of these means necessarily involve the reduction of the tetrachloride of the metal.

In this category may be mentioned particularly the process of British Patent No. 479,014 of January 28, 1938. According to this patent, molten sodium was floated on molten alkali halide and titanium tetrachloride was added. The process could be said to encompass titanium chloride broadly, which is in fact claimed in the patent. The product of this process, which was commercially used by the Deutsche Gold u. Silber Scheide Anstalt, was not cold ductile—a requirement for useful titanium metal. The reason for the failure of this process was recognized by Kroll and fully set forth in German Patent No. 674,625 of April 18, 1939, namely the reduction of  $TiCl_4$ , with alkali metals, is incomplete and the  $TiCl_3$  and  $TiCl_2$  formed contaminate the product and cannot be separated from it.

In my studies of the process I learned that the difficulties of alkali metal reduction as experienced by the Scheide Anstalt and by Kroll were due, as stated by Kroll, to the incomplete reduction of titanium chlorides by alkali metals or for that matter by alkaline earth metals including magnesium unless a special procedure such as that of Kroll is employed. I found that this incomplete reduction was due to an equilibrium in which the alkali or alkaline earth metal could be present in solution up to a fairly high concentration in the presence of titanium dichloride and titanium metal. This finding is expressed by the reaction



The existence of this equilibrium with a considerable displacement to the left is the scientific discovery which forms the basis of my present invention.

It will be clear that the Kroll process avoids the difficulties due to this equilibrium by avoiding the formation of  $TiCl_2$  and obtaining the direct reduction of  $TiCl_4$  by the reaction



2

By further study of the Reaction 1 above I found that the equilibrium in this reaction was such that the higher the concentration of  $TiCl_2$  the higher the concentration of sodium metal solution with which it would be in equilibrium.

For the purposes of my invention the reasons for this unique situation were not of any importance. I have found, however, in more recent studies of the processes of my invention that the activity of the alkali metal solution is a negative exponential function of its concentration. This leads to an equilibrium constant for Equation 1 of the form

$$(3) \log K = \log C_{TiCl_2} - nC_{Na^0}$$

15 This explanation is given here to enable those skilled in the art to better understand my invention.

In its broadest embodiment my invention consists in bringing a very dilute solution of a lower chloride of titanium or zirconium in a fused alkali or alkaline earth chloride into contact with a very dilute solution of an alkali or alkaline earth metal in a fused alkali or alkaline earth chloride.

I have found that the rate of diffusion of the alkali and alkaline earth metals is much greater than the rate of diffusion of lower titanium and zirconium chlorides dissolved in fused alkali or alkaline earth chlorides. Several embodiments of my invention are therefore based on control of the rate of diffusion of the alkali or alkaline earth metal which is being brought into contact with the solution of titanium chloride according to Reaction 1 above. It is a matter of relative simplicity to produce a concentration gradient of lower titanium chloride in a fused alkali or alkaline earth chloride. My invention includes several processes of doing this which will be illustrated. In the present example I simply add a solution of  $TiCl_2$  in  $LiCl-KCl$  eutectic which may be produced by methods I shall detail later.

I allow the concentration of the  $TiCl_2$  to attenuate to a few hundredths of a percent titanium by weight of the melt. I then add a dilute solution of lithium in the eutectic which can be produced by simple solution of the metal in the eutectic. The lithium solution is of comparable concentration to the titanium chloride. The titanium solution is added at exactly the same rate, stoichiometrically, as the lithium solution. I find that under these conditions there is formed at the outset pure particulate titanium at the point of addition of the lithium solution. However, with continued addition of the lithium solution the more rapid diffusion of the lithium causes the reaction zone to move toward higher concentrations of the titanium chloride which in accordance with Reaction 1 and Equation 3 brings about incomplete reduction of the titanium—a situation which grows worse like a chain-reaction. Equation 3 is in fact a mathematical expression of the conditions for a chain-reaction.

One embodiment of my invention, therefore, includes methods for preventing uncontrolled diffusion of the alkali or alkaline earth metal solution.

Briefly these methods include:

(a) Procedures for reaction preferentially with the alkali metal solution;

(b) Procedures which reduce the rate of diffusion of the alkali or alkaline earth metal in the fused bath.

In the simplest instance the procedure of "a" above may be followed by adding chlorine at a point where the diffusing alkali metal escapes from the reaction zone. This chlorine reacts preferentially with the dissolved alkali metal and with proper control need be added in only small amount as only the dissolved alkali metal escaping reaction with the titanium dichloride need be arrested. Of course the chlorine added represents a degree of inefficiency in reduction, but this is a small

price to pay for obtaining the titanium in particulate crystalline form.

While the reaction at the reaction zone is complete and the titanium formed is not contaminated with  $TiCl_2$  or  $TiCl_3$ , it is sometimes inconvenient to isolate this reaction zone from the zone of  $TiCl_2$  concentration. In such instances, I may first cease addition of the alkali or alkaline earth metal and the lower chloride of titanium and then add chlorine to convert all the  $TiCl_2$  to  $TiCl_3$  which can be leached from the particulate metal in only slightly acid solutions. Alternatively, I dissolve the salt containing  $TiCl_2$  in an acid solution containing an oxidizing agent, e. g.  $FeCl_3$ , which prevents the formation of the insoluble decomposition products of  $TiCl_2$ . In place of chlorine I may add  $TiCl_4$  and  $TiCl_3$  which serves the same purpose but less adequately because in such event some finely divided titanium is formed.

It must be noted here that my invention is not stepwise reduction of titanium chlorides, which is old as noted in British Patent No. 479,014 and German Patent No. 674,625, previously referred to. Stepwise reduction does not accomplish my result except perhaps transiently. My invention consists in preventing the alkali or alkaline earth metal from diffusing beyond the reaction area and reacting with relatively large concentrations of  $TiCl_2$ . My invention therefore requires a proper relationship between rate of addition of the reactants, in this instance titanium dichloride, alkali or alkaline earth metal and chlorine,  $TiCl_4$  or  $TiCl_3$ .

So far there have not been discussed procedures for adding the reactants other than simple addition which will be fully illustrated by examples.

Procedure "b" above encompasses methods of lowering the rate of diffusion of the alkali metal introduced into the fused halide bath. One method which I have found for accomplishing this is to select a reducing metal which is as little soluble as possible in the fused bath chosen. For example, I take a bath of  $KCl+NaCl$  and add a small amount of metallic barium which sinks to the bottom and dissolves only very slightly in this bath. I then add sodium to the barium and a chloride of titanium to the fused bath. Sodium being soluble in the barium diffuses slowly and meets the low concentration of diffusing titanium chloride a little above the barium layer. A foraminous barrier may be suitably placed above the barium layer so that the particulate titanium is deposited on it. Magnesium may be used in place of the barium. Since the magnesium floats the geometrical distribution of the foraminous barrier must be different. This will be illustrated by examples.

Other combinations for accomplishing the same thing include:  $KCl+LiCl+MgCl_2$ ;  $LiCl+SrCl_2$ .

In the following examples it will be understood that all procedures are carried out in accordance with accepted practice in the titanium industry. The metal and the fused salt bath are at all times protected with an inert atmosphere usually pure argon. It will also be understood that the temperatures of operation, which are not particularly critical, may be adjusted to the melting point of the bath to the end that the latter be maintained molten. In describing the constituents of the bath in this application I have used the term "alkaline metal chlorides," which term is meant to include the chlorides as well as the bromides of magnesium, barium, sodium, potassium, and lithium. It is also to be understood in every instance, except where noted, that zirconium may be substituted for titanium in carrying out the process of the example.

The invention will now be described in greater detail, and with reference to the accompanying drawing, in which:

Figure 1 is a diagrammatic representation of one form of non-electrolytic apparatus for use in carrying out a process according to the invention, showing one

arrangement of apparatus for retarding the rate of diffusion of reducer metal through a fused halide bath;

Figure 2 is a diagrammatic representation of a similar form of non-electrolytic apparatus, involving use of a horizontally disposed foraminous barrier member; and

Figure 3 is a diagrammatic representation of an electrolytic cell adapted for use in carrying out the process of the invention.

#### Example I

The reaction vessel for carrying out this example is illustrated in Figure 1. In this figure, 1 is a reaction vessel of steel provided with a cover 4, and inlet for argon 5, and an outlet for argon 6. The entire pot is surrounded with a furnace to maintain a temperature of  $850^{\circ}C$ . An open-bottom bell 2 passes through the cover. This bell is formed of titanium. A multiplicity of titanium tubes 3 are spaced peripherally around the bell so that they introduce  $TiCl_4$  into the reaction zone beneath and adjacent the open bottom of bell 2.

In this reaction vessel I react 46 lbs. of sodium with 188 lbs. of  $TiCl_4$  maintaining the temperature within the range of  $400^{\circ}-500^{\circ}C$ . and so that the reaction proceeds at a moderate rate. This produces essentially  $TiCl_2$  and sodium chloride. The reaction mixture is protected with argon in the closed reaction vessel. When the reaction is complete I add 5 times the amount of  $NaCl$ , and melt the mixture at  $850^{\circ}C$ , out of access to air. I now introduce a saturated solution of sodium in molten  $NaCl$  into a restricted area in the vessel defined by said bell, and add sodium within this restricted area. The reaction zone is maintained just outside the restricted area and at such a point that the concentration of sodium in the molten  $NaCl$  beneath the bell reaches  $.8 \times 10^{-3}$  gram equivalents per gram of fused salt. I add  $TiCl_4$  just outside the area, that is to say, to the salt bath adjacent the open bottom of the bell. In this way any dissolved sodium which escapes the reaction zone forms  $TiCl_2$ . The titanium metal formed in the reaction zone is pure crystalline Ti and agglomerates of filiform particles of Ti.

At the completion of the operation I continue to pass in  $TiCl_4$  until the sodium is entirely reacted and the residual  $TiCl_2$  is converted to  $TiCl_3$ . I then leach the salt from the Ti with very dilute acid.

#### Example II

I proceed as in Example I except that I substitute  $ZrCl_4$  for the  $TiCl_4$  in the initial reaction, and that vaporized  $ZrCl_4$  is passed into the reaction vessel through tubes 3. Coarsely crystalline zirconium is formed in the reaction zone.

#### Example III

I proceed as in Example I except that at the completion of the reaction I do not add excess  $TiCl_4$  but add magnesium to reduce the residual  $TiCl_2$  to Ti. I then wash with dilute acid to remove the salt.

#### Example IV

I proceed as in Example I except that at the completion of the reaction I do not add excess  $TiCl_4$  but dissolve the salt in a slightly acidified solution of ferric chloride to prevent the precipitation of insoluble titanium compounds.

#### Example V

I proceed as in Example II except that I pass chlorine into the reaction zone instead of  $ZrCl_4$ .

#### Example VI

I proceed as in Example I except that I use as the fused bath a eutectic mixture of  $KCl+NaCl$ . I then place a layer of magnesium in the bell and add sodium to the magnesium layer and  $TiCl_2$  to the periphery of the bath. I add these at a rate to bring the reaction zone to the place indicated in Figure 1. This is established as a steady

state under conditions where the concentration of sodium reaching the reaction zone is below  $10^{-3}$  gram equivalents per gram and the titanium dichloride concentration reaching the reaction zone is also less than  $10^{-3}$  gram equivalents per gram of fused salt.

#### Example VII

I proceed as in Example VI except that I add  $TiCl_4$  at the outer periphery of the reaction zone.

#### Example VIII

In this example I place a layer of barium on the bottom of a reaction vessel and use a bath of sodium and potassium chloride. I place over this layer of barium a foraminous barrier. I pass sodium into the barium layer. I then produce  $TiCl_2 + TiCl_3$  in the upper portion of the bath by reacting sodium with  $TiCl_4$ . I cause this mixture to diffuse downward and meet the upwardly diffusing sodium just above the foraminous barrier. The titanium collects on the foraminous barrier which is conveniently made of Ti. At the end of the reaction I add an excess of  $TiCl_4$  and then drain off the salt from the bottom of the vessel leaving the titanium mixed with some salt on the foraminous barrier. The titanium salt in this mixture is  $TiCl_3$ . I remove the salt by washing with very dilute HCl.

Figure 2 illustrates an apparatus for carrying out an embodiment of this invention. In this figure, A represents a steel pot with a bottom outlet B connected to a similar pot (not shown) by a pipe C and means (not shown) for transfer of liquids between pots. The pot is provided with a cover D and with an inlet E and outlet F to provide an argon atmosphere within the pot. The pot is filled with NaCl-KCl mixture and this mixture is fused. The bottom outlet B is frozen and a layer of barium Ba placed on the bottom. A foraminous titanium screen G is put in place above the barium layer, and a tube H arranged for feeding sodium into the barium layer. Two tubes J and K are provided through the cover for introducing sodium and  $TiCl_4$ , respectively.

The  $TiCl_2$  formed is caused to diffuse downward to meet the upwardly diffusing sodium. These reactants are caused to meet at low concentration just above the foraminous barrier G. The location of this reaction zone is regulated by the rate of addition of the sodium to the barium layer and the rate of addition of the  $TiCl_4$  and Na in the upper part of the bath. When the proper steady state is established the  $TiCl_4$  and total sodium must be in stoichiometric proportions to form Ti.

The amount of barium is also a factor as the sodium alloyed must not cause it to float.

#### Example IX

In this example I set up an electrolytic cell with an electrolyte of fused sodium chloride. I place the two electrodes at a distance of 1 foot and I add 1% by weight of  $TiCl_2$  to the bath. I then pass a unidirectional current from a metallic Ti anode to a steel cathode at such a current density that the diffusion of  $TiCl_2$  from the anode when established at a steady rate just maintains the concentration at the cathode of 0.1% by weight. I then remove the cathode plate with adhering titanium crystals and wash with water to remove the salt. The crystals obtained in this way are melted in an arc furnace in an inert atmosphere and have a Brinell hardness of 80.

#### Example X

I proceed as in Example IX except that I use an impure titanium anode containing oxygen and iron and having a Brinell hardness of 250. The recovered titanium is fully refined and has a Brinell hardness of 80.

#### Example XI

I proceed as in Example IX except that I add  $Cl_2$  near the cathode. As a result I increase the current density at which the necessary steady state of concentration is ob-

tained. The result so far as producing titanium is the same. At the end of the run I pass enough chlorine into the bath to convert  $TiCl_2$  in the bath to  $TiCl_3$ . I then remove the cathode and dissolve the salt.

#### Example XII

In this example I use an impure zirconium anode and a pure zirconium cathode. I use an electrolyte of 35% KCl, 35% NaCl, 30%  $BaCl_2$ . I pass a unidirectional current until the open circuit voltage of the cell reaches 0.5 volt. I then add chlorine to reduce this voltage to 0.1 volt and continue electrolysis. I proceed in this fashion with periodic additions of chlorine. I use for this purpose an electrolytic cell like that of Fig. 3.

In Figure 3 an iron pot A is provided with a bottom outlet B, a cover C, and argon inlet D and outlet E. In this pot is a liner F with a foraminous bottom F'. This serves as a cathode. An anode G of crude titanium is inserted centrally in the pot and immediately below the anode is an anode slime cup H to catch the anode slime.

The crystalline zirconium is deposited on the titanium liner F and F' and at the end of the run the salt is withdrawn from the bottom of the pot and the titanium recovered from the liner by dissolving in dilute HCl containing  $FeCl_3$ .

#### Example XIII

In this example I produce an adherent continuous non-porous plate of titanium on steel by making the steel a cathode in an electrolytic cell having a titanium anode and an electrolyte of 40% KCl, 40% NaCl and 20%  $BaCl_2$ . I pass a unidirectional current through the cell at 1 ampere per square inch until the open circuit voltage of the cell reaches 0.1 volt. I then interrupt the electrolysis, and regenerate the electrolyte by adding chlorine. This cycle is repeated until the desired thickness of plate is obtained.

#### Example XIV

In this example I use an electrolytic cell with an anode of impure titanium, the electrolyte is fused  $MgCl_2$  at  $850^\circ C$ . with 5% added  $TiCl_2$ . The cathode is a rotating titanium disc. When a current of 1000 amperes/sq. ft. is passed through this cell, an open circuit voltage of 0.9 volt is soon found. This clearly corresponds to deposition of magnesium with some titanium at the cathode. I now add  $Cl_2$  until the open circuit voltage of the cell is less than 0.1 volt which indicates that there is substantially no codeposition of Mg with the Ti, and then proceed with the electrolysis with the necessary additions of  $Cl_2$ . It will be clear that under these circumstances the titanium chloride content of the bath is increasing. To obviate this I add magnesium periodically. If the magnesium is added in exactly an amount equivalent to the  $Cl_2$  then the titanium chloride in the bath will remain constant and only the  $MgCl_2$  will increase. The magnesium must not be added in such amounts as to form titanium metal but only to reduce  $TiCl_3$  to  $TiCl_2$ . This may be balanced against the withdrawal on the cathode. Since the cell of this example is a continuous arrangement, the withdrawn metal attached to the cathode contains  $MgCl_2$  and  $TiCl_2$ . These salts cannot be effectively removed by water washing so that I remove them by pressing and evaporation as set forth, for example, in my copending application Serial 391,153, filed November 9, 1953. The final product is a pure titanium ingot with a hardness of Brinell 90.

#### Example XV

I proceed as in Example XIV except that I use a crude zirconium anode and an electrolytic bath of 50%  $CaCl_2$  and 50% NaCl at  $650^\circ C$ . The original open circuit voltage of the cell is 1.4. Sodium is added directly to the cell periodically in an amount equivalent to the chlorine necessary to maintain the voltage at 0.1 volt. The sodium is added at regular intervals and only in such amounts as to reduce  $ZrCl_3$  to  $ZrCl_2$  and not to form zirconium metal.

In this example the salts including the zirconium chlorides may be dissolved from the metal by an acid solution of ferric chloride.

I claim:

1. In a process for the production of a crystalline deposit of a metal of a first group consisting of titanium and zirconium by reduction of a lower chloride of a metal of said first group in solution in a fused bath of at least one salt selected from the group consisting of alkali metal chlorides, alkaline earth metal chlorides and magnesium chloride by reaction therewith of a reducer metal selected from the group consisting of alkali metals, alkaline earth metals and magnesium dissolved in a fused bath of at least one salt selected from the group consisting of alkali metal chlorides, alkaline earth metal chlorides and magnesium chloride, the steps which consist in bringing together said solution of the chloride of said first group metal and said solution of reducer metal in a reaction zone at a low concentration of both reactants below  $10^{-3}$  gram equivalents per gram of said fused salt and thereafter adding said solutions of reactants to the reaction zone at rates which maintain such low concentration and in stoichiometric proportions whereby said first group metal is produced in coarsely crystalline form.

2. In a process for the production of a crystalline deposit of a metal of a first group consisting of titanium and zirconium by reduction of a chloride of a metal of said first group by reacting (1) a solution of a lower chloride of said first group metal in a fused bath of at least one salt of the group consisting of alkali metal chlorides and bromides, alkaline earth metal chlorides

and bromides, magnesium chloride and magnesium bromide, with (2) a solution of a reducer metal of the group consisting of alkali metals, alkaline earth metals and magnesium in a fused bath of at least one salt of the

5 group consisting of alkali metal chlorides and bromides, alkaline earth metal chlorides and bromides, magnesium chloride and magnesium bromide, the step which consists in maintaining in the zone of the reaction a concentration of both reactants at below  $10^{-3}$  gram equivalents per 10 gram of said fused salt by adding said solution of lower chloride of metal of the first group and said solution of reducer metal to the reaction zone at a rate which maintains such concentration.

15

References Cited in the file of this patent

UNITED STATES PATENTS

|           |                |               |
|-----------|----------------|---------------|
| 2,148,345 | Freudenberg    | Feb. 21, 1939 |
| 2,205,854 | Kroll          | June 25, 1940 |
| 2,561,862 | Hill           | July 24, 1951 |
| 2,607,674 | Winter         | Aug. 19, 1952 |
| 2,722,509 | Wainer         | Nov. 1, 1955  |
| 2,734,855 | Buck et al.    | Feb. 14, 1956 |
| 2,734,856 | Schultz et al. | Feb. 14, 1956 |
| 2,783,196 | Raney          | Feb. 26, 1957 |

FOREIGN PATENTS

|         |               |               |
|---------|---------------|---------------|
| 682,919 | Great Britain | Nov. 19, 1952 |
|---------|---------------|---------------|

OTHER REFERENCES

30 Sibert et al.: "Electrolytic Titanium," Journal of Metals, September 1956, pages 1162-1168.